

## UNITED STATES PATENT OFFICE.

ANDREW O'ROURKE, OF CHICAGO, ILLINOIS, ASSIGNOR TO CRANE COMPANY, OF CHICAGO, ILLINOIS, A CORPORATION OF ILLINOIS.

## ALLOY.

No Drawing.

Application filed February 27, 1922. Serial No. 539,758.

To all whom it may concern:

Be it known that I, ANDREW O'ROURKE, a citizen of the United States, residing at Chicago, in the county of Cook and State 5 of Illinois, have invented a new and Improved Alloy, of which the following is a full, clear, and exact description:

This invention relates in general to alloys, and has for its primary purpose the production of a new and improved alloy which is 10 particularly suitable for the manufacture of plumbing fixtures, valve discs, valve casings, and the like.

Fixtures of this character have heretofore 15 customarily been nickel-plated to give them the desired luster and appearance. My improved alloy however obviates the labor and expense of nickel-plating since the alloy itself from which the articles are formed 20 possesses the capability of taking a high polish so as to present a luster which closely simulates in appearance nickel-plating. Furthermore, the alloy is adapted to retain this luster to a very high degree without 25 tending to tarnish, and, in addition, since an article made from this alloy is homogeneous throughout, there is no liability of the luster being worn off by prolonged usage so 30 as to detract from the pleasing appearance of the article as frequently occurs in nickel-plated articles when the plating wears or chips off.

An alloy made in accordance with my invention is composed of metals in substantially the following proportions.

|                | Per cent. |
|----------------|-----------|
| Copper -----   | 50 to 65  |
| Zinc -----     | 8 to 20   |
| Nickel -----   | 10 to 25  |
| 40 Lead -----  | 3 to 10   |
| Tin -----      | 1 to 5    |
| Antimony ----- | 5 to 2    |
| Iron -----     | 0 to 2    |

45 While variations in the proportions of the ingredients will impart to the alloy different characteristics as to hardness, strength, ductility, etc., I have found that proportions within the ranges above specified are 50 suitable for the various articles which I contemplate manufacturing therefrom. The ingredients are melted together to form the

alloy which can be poured while molten into molds in which it is cast into the desired form. The resultant product is nearly white 55 in color, approximating closely to the color of nickel, and it is sufficiently soft to enable it to be readily and rapidly machined. After the machining operations, if the character of the article requires machine work, 60 the surfaces of the article may be polished in any well known or preferred manner, and as the result of the polishing operation and without depositing thereon any coating or plating whatsoever, the article takes on a 65 high luster closely resembling nickel-plating in appearance, which luster it will retain without tendency to tarnish.

While in most instances no iron whatever or only a trace is employed, I have found 70 that a small quantity thereof is not detrimental and for some articles is advantageous. The antimony lends itself to the capabilities of the alloy to assume a high polish and present a lustrous appearance, but since 75 larger quantities of antimony tend to make the alloy more brittle and difficult to machine, I prefer to restrict the quantity of this ingredient substantially within the limits above specified.

80 It should be apparent from the foregoing that I have provided an alloy possessing highly desirable properties and capable of many uses, and it should be manifest that a considerable range in proportions of the 85 various ingredients may be invoked within the scope of my invention as defined in the following claims.

I claim:

1. An alloy, consisting of the following 90 ingredients in substantially the proportions specified: copper 50 to 65 per cent; zinc 8 to 20 per cent; nickel 10 to 25 per cent; lead 3 to 10 per cent; tin 1 to 5 per cent, and antimony  $\frac{1}{2}$  to 2 per cent.

95 2. An alloy adapted to receive a high polish and consisting of the following ingredients in substantially the proportions specified: copper 50 to 65 per cent; zinc 8 to 20 per cent; nickel 10 to 25 per cent; lead 100 3 to 10 per cent; tin 1 to 5 per cent; antimony  $\frac{1}{2}$  to 2 per cent, and iron in substantial amount, but not over 2 per cent.

ANDREW O'ROURKE.

7

**Certificate of Correction.**

It is hereby certified that in Letters Patent No. 1,448,571, granted March 13, 1923, upon the application of Andrew O'Rourke, of Chicago, Illinois, for an improvement in "Alloys," an error appears in the printed specification requiring correction as follows: Page 1, line 42, for the numeral "5" read ".5"; and that the said Letters Patent should be read with this correction therein that the same may conform to the record of the case in the Patent Office.

Signed and sealed this 3d day of April, A. D., 1923.

KARL FENNING,

*Acting Commissioner of Patents.*

[SEAL.]